# EUROPEAN PATENT SPECIFICATION

(11) **EP 0 648 689 B1**
(45) Date of publication and mention of the grant of the patent: **09.04.1997**
(21) Application number: 94307360.1
(22) Date of filing: 06.10.1994
(51) Int. Cl.: B65D 81/28, D21H 21/36

(54) **Packaging of cleaning products**
Verpackung für Reinigungsprodukte
Emballage pour des produits de nettoyage

(30) Priority: 06.10.1993 GB 9320604
(43) Date of publication of application: 19.04.1995
(73) Proprietor: MORRIS GREENHALGH LIMITED, Bolton BL1 2NP (GB)
(72) Inventor: Wood, Stephen Graham, Bolton BL1 2NP (GB)
(74) Representative: Atkinson, Peter Birch

(56) References cited:
- FR-A- 2 016 071
- US-A- 3 270 022
- PATENT ABSTRACTS OF JAPAN vol. 16, no. 273 (C-0953) 18 June 1992 & JP-A-04 069 301 (OHBAYASHI CORP.) 4 March 1992
- DATABASE WPI Week 9303, Derwent Publications Ltd., London, GB; AN 93-019003 & DE-A-41 22 654 (BAYER AG) 14 January 1993

## Description

The present invention relates to the packaging of cleaning products as well as to materials useful as packaging.

Examples of cleaning products with which the invention is concerned includes personal care products such as tablets of soap as well as domestic cleaning products such as detergent formulations for laundering or dishwashing purposes.

Various types of packaging are used for cleaning products. For example, soap tablets are wrapped in paper and as a further example detergent powders are packaged in cardboard boxes. As an additional example, liquid cleaning products (e.g. shampoos, dishwashing liquids) are sold in plastics containers. (The term packaging as used herein is also intended to cover such containers).

It has long been recognised that the components present in cleaning products encourage mould growth in or on the packaging material. Thus for example soap tablets generally have a relatively high moisture content and also contain fatty acids. This combination of moisture and fatty acids (which are mould nutrients) can lead to mould growth on the paper in which the soap is wrapped.

In order to avoid the problem of mould growth it has previously been proposed to incorporate a fungicide in the packaging material. One fungicide which has been used extensively for this purpose is Carbendazim.

Carbendazim does however have a number of disadvantages. In particular, it is classified as a pesticide which places restriction on its use and moreover does not provide a sufficiently wide spectrum of activity to give total protection against mould growth.

Another fungicide which has been used in packaging for cleaning products is TCMTB but this sensitises skin.

JP900180462 discloses the use of pyrithione compounds in the treatment of paper for use in the construction of building boards. DE4122654 describes a composition containing a pyrithione compound used for the treatment of wood.

It is therefore an object of the present invention to obviate or mitigate the abovementioned disadvantages.

According to a first aspect of the present invention there is provided the combination of a cleaning product enclosed within packaging which incorporates a fungicidally effective amount of a pyrithione derivative, wherein the pyrithione derivative has a particle size of less than 10 microns.

The cleaning product may for example be a solid product such as a tablet of soap (wrapped within packaging incorporating the pyrithione derivative) or a detergent powder in a box formed of a material incorporating the pyrithione derivative. Alternatively the cleaning product may be a liquid provided in a plastics container whereof the plastics material incorporates the pyrithione derivative.

Pyrithione is a compound of the following structural formula

Other names for pyrithione include:
2-mercaptopyridine-N-oxide
1-hydroxypyridine-2-thione
2-pyridinethiol-1-oxide
1-hydroxy-2(1H)-pyridinethione

Pyrithione derivatives are used in a variety of personal care and cosmetic applications. Thus pyrithione derivatives are used as anti-dandruff agents m shampoos. As such, they are recognised as being non-harmful to human beings and therefore their use (as fungicidal agents in packaging for cleaning products) is fully acceptable.

The pyrithione derivative is preferably incorporated in the packing material in the form of particles having a size of less than 5 microns. Preferably the packaging material comprises 250-2000 ppm of the pyrithione derivative. The pyrithione derivative may be incorporated in the base material of the packaging either during or after its production.

The pyrithione derivative used in the invention is most preferably an insoluble derivative so as not to be "washed" off the packaging of the packaged cleaning product if the product is stored under conditions in which condensation is generated.

The preferred pyrithione derivative for use in the invention is zinc pyrithione which is of the formula:

This compound is available from Olin Corporation under the trade mark Zinc Omadine.

One example of packaging material is a non-woven cellulosic product, e.g. paper, cardboard or the like (such materials are particularly suitable for the packaging of solid cleaning products, e.g. soap tablets, powdered detergents). The pyrithione may be incorporated in the suspension of cellulose fibres from which the paper (or the like) web is formed. Alternatively the pyrithione derivative may be applied after formation of the web, e.g. by incorporating the pyrithione derivative in a solution (e.g. a thin starch solution) to be applied to the web at a size press, coating station or callender box.

The invention will be illustrated by the following non-limiting Example.

### Example

Two identical samples of paper were taken and one was treated with 750 ppm Zinc Omadine, the other being untreated to serve as a control.

The paper samples were then placed on nutrient agar, sprayed with a mixed fungal suspension, and observed over a period of six weeks for fungal growth.

The untreated paper was found to be completely overgrown by fungus after 1 week whereas there was no fungal growth on the paper treated with Zinc Omadine even after six weeks.

Zinc Omadine treated paper is therefore eminently suitable for use in wrapping soap tablets.

## Claims

1. A solid cleaning product enclosed within packaging which incorporates a fungicidally effective amount of a pyrithione derivative, wherein the pyrithione derivative has a particle size of less than 10 microns.

2. The combination as claimed in claim 1 wherein the pyrithione derivative is an insoluble derivative.

3. The combination as claimed in claim 1 wherein the pyrithione derivative is zinc pyrithione.

4. The combination as claimed in any one of claims 1 to 3 wherein the pyrithione derivative has a particle size of less than 5 microns.

5. The combination as claimed in any one of claims 1 to 4 wherein the packaging material comprises 250-2000 ppm of the pyrithione derivative.

6. The combination as claimed in any one of claims 1 to 5 wherein the packaging material is a non-woven cellulosic product.

7. The combination as claimed in any one of claims 1 to 6 wherein the cleaning product is a tablet of soap.

8. The combination as claimed in any one of claims 1 to 6 wherein the cleaning product is a powdered detergent.

## Patentansprüche

1. Festes Reinigungsmittel, das von Verpackung umgeben ist, welche eine pilztötende Menge eines Pyrithionderivates enthält, wobei das Pyrithionderivat eine Teilchengröße von weniger als 10 Mikron hat.

2. Kombination nach Anspruch 1, bei der das Pyrithionderivat ein unlösliches Derivat ist.

3. Kombination nach Anspruch 1, bei der das Pyrithionderivat Zinkpyrithion ist.

4. Kombination nach irgendeinem der Ansprüche 1 bis 3, bei der das Pyrithionderivat eine Teilchengröße von weniger als 5 Mikron hat.

5. Kombination nach irgendeinem der Ansprüche 1 bis 4, bei der das Verpackungsmaterial 250 - 2000 ppm des Pyrithionderivates enthält.

6. Kombination nach irgendeinem der Ansprüche 1 bis 5, bei der das Verpackungsmaterial ein nichtgewebtes Zelluloseprodukt ist.

7. Kombination nach irgendeinem der Ansprüche 1 bis 6, bei der das Reinigungsmittel ein Seifenstück ist.

8. Kombination nach irgendeinem der Ansprüche 1 bis 6, bei der das Reinigungsmittel ein Detergenspulver ist.

## Revendications

1. Produit de nettoyage solide renfermé dans un conditionnement dans lequel est incorporée une quantité efficace à effet fongicide d'un dérivé de pyrithione, dans lequel le dérivé de pyrithione possède une granulométrie inférieure à 10 microns.

2. Combinaison selon la revendication 1, dans laquelle le dérivé de pyrithione est un dérivé insoluble.

3. Combinaison selon la revendication 1, dans laquelle le dérivé de pyrithione est la pyrithione de zinc.

4. Combinaison selon l'une quelconque des revendications 1 à 3, dans laquelle le dérivé de pyrithione possède une granulométrie inférieure à 5 microns.

5. Combinaison selon l'une quelconque des revendications 1 à 4, dans laquelle la matière de conditionnement comprend 250-2000 ppm du dérivé de pyrithione.

6. Combinaison selon l'une quelconque des revendications 1 à 5, dans laquelle la matière de conditionnement est un produit cellulosique non tissé.

7. Combinaison selon l'une quelconque des revendications 1 à 6, dans laquelle le produit de nettoyage est un pain de savon.

8. Combinaison selon l'une quelconque des revendications 1 à 6, dans laquelle le produit de nettoyage est un détergent pulvérulent.
